# EUROPEAN PATENT APPLICATION

(11) **EP 0 269 440 A1**
(43) Date of publication of application: **01.06.1988**
(21) Application number: 87310424.4
(22) Date of filing: 25.11.1987
(51) Int. Cl.: B41M 5/26

(54) **Multicolor heat-sensitive recording material**

(30) Priority: 26.11.1986 JP 282789/86
(71) Applicant: Fuji Photo Film Co., Ltd., Kanagawa-ken (JP)
(72) Inventor: Washizu, Shintaro, Fujinomiya-shi Shizuoka 418 (JP); Usami, Toshimasa, Fujinomiya-shi Shizuoka 418 (JP); Tatsuta, Sumitaka, Fujinomiya-shi Shizuoka 418 (JP)
(74) Representative: Diamond, Bryan Clive (GB)

(57) **Abstract**

A transparent support, e.g. a plastics film, is coated with two or more layers (C, M and Y) producing different color hues, at least one of which is situate on each face of the support; each layer is composed of a combination of
(a) a precursor (usually nearly colorless) of a basic dye and
(b) an electron accepting color developer (e.g. a phenol),
(c) a diazo compound (diazonium salt) and
(d) a coupler therefor.
These components are preferably microencapsulated in various combinations.

A compound which assists the color formation upon heating can be added; a subbing layer and/or overcoat layer can be present.

Recording by heat from a thermal head on one or both surfaces produces a dye and diazo image, and a wide range of color hues can be formed by imaging in the different color producing layers.

## Description

The present invention relates to a heat-sensitive recording material which can record many colors

In more detail, it is concerned with a multicolor heat-sensitive recording material which enables substantially independent heat recording of several images differing in hue.

A heat-sensitive recording method has many advantages, in that
(1) no particular developing step is required,
(2) if paper is used as a support, the recording material prepared can have a quality akin to that of plain paper,
(3) the handling of a recording material used is easy,
(4) images recorded have high color density,
(5) this method can be carried out using a simple and cheap apparatus, and
(6) no noise is generated upon recording.
Therefore, heat-sensitive recording materials have recently come into wide use for use with black and white facsimile machines and printers. These heat-sensitive recording materials are prepared by coating a combination of a color producing agent and a color developing agent on a support, such as paper or synthetic paper, and a record is made thereon through a process of heating with a thermal head on the basis of electric signals corresponding to an original.

In the above-described recording fields also, a requirement to get colored hard copies with ease from data terminals of information equipment such as a computer or a facsimile has increased with the rapid advance of the information industry. As a method of fulfilling such a requirement, an ink jet process and a heat-sensitive transfer process have been considered. In the ink jet process, however, a coloring agent and other ingredients in ink tend to cause stopping-up of a nozzle because of the narrowness of the nozzle out of which the coloring agent-containing ink is shot. Therefore, such a process has a serious defect that it lacks reliability of the records formed. In the heat-sensitive transfer process, on the other hand, ink on an ink sheet is dissolved imagewise by heating, and transferred onto paper. Accordingly, in order to obtain, for example, a 4-color image four ink sheets, are required. Such a process is uneconomical since it requires a great number of ink sheets. In addition, a user must devote ceaseless attention so that ink solutions, in case of the ink jet process, and ink sheets, in case of the heat-sensitive transfer process, do not become scarce in supply. That is to say, both the processes require bothersome supervision by users.

In contrast to the foregoing processes, a heat-sensitive recording process requires no bothersome supervision, and can provide highly reliable records. Therefore, when a multicolor recording material is used in this process, the material can be free from the defects of conventional processes, and used with ease. In order to render a record multicolored, however, it is necessary to provide, on one support, color-producing mechanisms in number corresponding to that of the colors to be produced, and to make the color-producing mechanisms fulfil their respective functions under control. Although much efforts to meet the above-described requirements have so far been made, all materials proposed are still insufficient in respect of hue and color separation of produced colors.

For instance, there is a conventional method in which several colored units are simply added one after another in proportion as applied heat energy is increased, and thereby the produced colors are mixed, to cause changes in hue accompanied by turbidity, as described in Japanese Patent Publications Nos. 19989/76 and 11231/77, and Japanese Patent Applications (OPI) Nos.88135/79, 133991/80 and 133992/80(The term "OPI"as used herein means an unexamined published application ). As another conventional method, there is known one which introduces decolorization mechanisms, such that a color produced by a color-producing unit at a low temperature is decolorized by the reaction with a decolorizing agent at the same time as a color-producing unit capable of making a thermal response at a higher temperature produces its color, as described, e.g., in Japanese Patent Publications Nos. 17868/75, 5791/76, 14318/82 and 14319/82, and Japanese Patent Application (OPI) No.161688/80.

In the above-described methods, not only is the number of realizable hues small, but also turbidity due to blur and color mixing is generated. Therefore, the heat sensitive materials employed in the foregoing methods do not serve very well for producing a color hard copy. In particular, it is a fatal defect for a color hard copy that the number of hues of producible colors is in principle small. One material reason why the conquest of this defect has not yet been successful is due to the following circumstances. That is, if an increase in number of producible hues can be achieved by simply increasing the number of fractions of heat energy applied for printing and, at the same time, making a large difference in energy between one fraction and another one, it suffices in principle for this purpose to design a heat-sensitive recording material provided with an increased number of heat-sensitive color-producing layers on the same support so as to correspond to various heat energies applied thereto respectively. In reality, however, there occur problems in respect of the freshness keeping property (the so-called fog) of the recording material itself, when heat energy applied for printing is extended to a lower region than usual, while when the energy is extended to a higher region, there arise new grave problems that images formed become sticky through their burning or fusion (e.g., a sticking phenomenon tends to occur), whereby the travelling facility of a thermal head upon printing is deteriorated, the span of thermal-head life becomes short, and so on. Accordingly, the largest allowable number of fractions of heat energy to be applied for printing has so far been two or so from the practical viewpoint of satisfactory color separation.

In the meantime, an opaque support, such as paper, synthetic paper or the like, has usually been employed as the support of a heat-sensitive recording material. This merely allows the customary use of the produced color images as reflected images to be read from one side.

As hitherto known examples of a heat-sensitive recording material provided with a substantially transparent support, mention may be made of those described in Japanese Patent Application Nos. 68875/85 and 184483/85. Therein, the transparent support was used for the purpose of obtaining a high quality image, especially excellent in luster, by observing the images recorded by heat from the side of the transparent support. In addition, " dichromatic heat-sensitive paper having a highly transparent base material, e.g., some kind of synthetic resin film or paper, which is provided respectively on both sides with layers containing heat-sensitive recording agents differing in hue of recorded image" is reported in Japanese Patent Application (OPI) No. 3640/75, and "dichromatic recording type heat-sensitive recording sheet characterized by heat-sensitive recording layers, in which different combinations of a diazo compound and a coupling component are contained respectively, provided on respective sides of a transparent base material" is reported in Japanese Patent Application (OPI) No. 4092/85. That is, attempts to form a dichromatic image by providing color-producing unit layers different in hue of produced color on both sides of a transparent support, respectively, have also been made. As noted previously, however, formation of several color-producing unit layers on the same side of a support causes a problem concerning the freshness keeping property (so-called fog) of the resultant heat-sensitive recording material. Therefore, any multicolored (including tricolored) heat-sensitive recording material excellent in hue and color separation has not been provided as yet.

Still another example of providing heat-sensitive color-producing layers on both sides of a support is disclosed in Japanese Patent Application (OPI) No. 208298/82. This aims at reduction of loss in aspects of cost, keeping space of printed copies, and so on by printing records on both sides of an opaque support. Accordingly, all the materials cited above do not have any special contribution to obviation of the foregoing defects inherent in multicolored recording material.

As the results of our energies research on the above-described problems, it has been found that when several color-producing layers differing in hue to be provided on both sides of a transparent support are constituted by not only layers containing as a color-producing unit a combination of a diazo compound with a coupling component, but also layers containing as a color-producing unit a combination of a basic dye precursor with a color developing agent, not only selection of color-producing agents becomes easy, and in its turn an advantage from the production point of view is greatly increased, but also a multicolor heat-sensitive recording material improved in freshness keeping property and image density to a satisfactory extent can be obtained.

Therefore, a first object of the present invention is to provide a multicolor heat-sensitive recording material having excellent freshness keeping property.

A second object of the present invention is to provide a multicolor heat-sensitive recording material excellent in density of the produced colors and other qualities.

A third object of the present invention is to provide a method of producing a multicolor heat-sensitive recording material superior in quality through extension of the range from which color-producing agents can be chosen.

The above-described objects are attained with a multicolor heat-sensitive recording material which comprises a transparent support having two or more of color-producing unit layers differing in hue of the produced color in such a situation that at least one unit layer is provided on each side of the support, with the unit layers being constituted by one or more of a color-producing unit layer containing a combination of a basic dye precursor with a color-developing agent as a color-unit, and one or more of a color-producing unit layer containing a combination of a diazo compound with a coupler as a color-producing unit.

In accordance with the present invention, the hue, color separation and color density of the multicolor image obtained are more excellent than conventional heat sensitive recording methods have ever provided. In addition, the image obtained is superior in keeping quality. Further, the invention makes it feasible to observe images as not only transmitted image, but also reflected image. Thus, the invention opens the way to forming natural color images by nonsilver photography, and has considerable significance.

In an embodiment of the multicolor heat-sensitive recording material (abbreviated as heat sensitive material, hereinafter) of the present invention, for instance, a transparent support provided with a transparent subbing layer on each side is used, and in forming on each of the subbing layers one or more of a heat sensitive layer (i.e., at least two or more of heat sensitive layers as a whole, which are different from one another in hue of the produced color), a color-producing unit layer containing a combination of a diazo compound and a coupling component as a color-producing unit is employed as one heat sensitive layer and a color-producing unit layer containing a combination of a basic dye precursor and a color developing agent as a color-producing unit is employed as another heat sensitive layer, and they are laminated as adjacent layers, followed by formation of an overcoat layer on each of the topmost heat sensitive layer.

As described above, a range of choice in color-forming agents can be extended by using diazo compounds and basic dye precursors in combination as color-forming agents. Further, the combined use of the foregoing color-forming agents is not only important from the standpoint of increasing numbers of producible colors, but also has an advantage in that the advantages gained from the use of basic dye precursor as color forming agent, that is, excellent keeping property and high color density of the produced image, can be utilized effectively.

A method for obtaining easily multicolor images of good quality by the use of the heat-sensitive recording material of the present invention is illustrated in the figures.
Fig. 1 and Fig. 3 are sectional views illustrating examples of heat sensitive materials having three color-producing layers in accordance with the present invention; and
Fig. 2 is a sectional view illustrating an example of the coloration caused in the heat sensitive material shown in Fig. 1 when thermal printing was carried out.

Fig. 1 shows an example of the heat sensitive material of the present invention, wherein on one side of a transparent supports is provided a cyan color-producing layer C containing a combination of a basic dye precursor with a color developing agent, while on the opposite side a yellow color-producing layer Y containing a combination of a diazo compound with a coupling compound is superposed on a magenta color-producing layer M.

In this case, it is desired from the standpoint of independent production of the third color that a system for carrying out both color-producing coupling reaction and photo-fixation reaction of a diazo compound, as described in Japanese Patent Application (OPI) No. 40192/86, should be introduced into either the yellow or magenta color-producing layer, e.g., a layer Y. More specifically, the yellow color- and cyan color-producing layers are firstly made to produce their respective colors at rather low temperature by recording of low thermal energy, and secondly photo-fixation is carried out using a light source of particular wavelengths which enable selective photolysis of only the diazo compound contained in the yellow layer, and then heat recording is made on the thermally low sensitive magenta layer by application of relatively high thermal energy compared with the preceding heat recording. Thus, cyan, magenta and yellow colors are produced independently on both sides of the support. When the resultant heat sensitive material is observed from one side of the transparent support, seven basic colors, i.e., cyan, magenta, yellow, cyan + magenta (blue), magenta + yellow (red), cyan + yellow (green), and cyan + magenta + yellow (black), can be produced therein in a good condition of color separation, hitherto regarded as difficult in heat sensitive recording.

In Fig. 2, the areas marked 1 to 7 designate respect tively the green, yellow, red, black, blue, cyan and magenta hues due to the colors shown produced in the three layers C, M and Y.

Alternatively, the heat sensitive material of the invention can be constituted in accordance with the embodiment shown in Fig. 3, wherein one side of a transparent support is provided a magenta color-producing layer M containing a combination of a diazo compound with a coupling compound as a color-producing unit, while on the opposite side are provided a cyan color-producing layer C containing a combination of a basic dye precursor with a color developing agent as a color-producing unit, and a yellow color-producing layer Y containing a combination of a diazo compound with a coupling component as color-producing unit, in this order.

It is again advantageous to introduce into the magenta color-producing layer and the yellow color-producing layer. More specifically, the heat recording process, in analogy with the heat sensitive material shown in Fig. 1, comprises, in the first place, producing colors in the magenta color- and yellow color-producing layers, respectively, by heat recording with rather low thermal energy, in the second place carrying out photofixation of the diazo compounds contained in the magenta color- and yellow color producing layers, and then carrying out recording on the cyan layer by applying thermal energy relatively higher than in the preceding recording, whereby achieving multicolor heat sensitive recording.

Numbers of colors producible by color mixing can be enlarged in a multiple manner by controlling the color-production in each unit through proper adjustment of heating energy for printing. This matter can be easily understood by those skilled in the art.

In order to obtain clearer hue in the heat recording, it is to be desired that each color-producing unit layer should be transparent in a substantial sense.

As for the processes of multicolor production in the present invention, brief illustration is given above. Now, detailed description of materials to be used for the multicolor heat-sensitive recording material of the present invention is given, especially as to the color-producing unit layers comprising a combination of a diazo compound with a coupling compound, and those comprising a combination of a basic dye precursor with a color developing agent.

The diazo compounds to be used as color forming agent in the present invention are those capable of forming colors of desired hues by reacting with coupling components described hereinafter, but decomposing on exposure to light of particular wavelengths prior to the coupling reaction to lose their color-forming ability, that is, to no longer form colors by making coupling components act thereon. The hue obtained in such a color-producing system depends mainly on the diazo dye produced by the reaction of a diazo compound with a coupling component. Consequently, as is well known, the hue of color to be produced can be changed with ease by modifying the chemical structure of diazo compound, and/or that of a coupling component. Almost any desired hue can be obtained depending on how the colors are combined. Therefore, one kind of coupling component and other additives may be incorporated in one layer in which various kinds of diazo compounds are dispersed. In this case, individual color-producing units are constituted with a diazo compound different from each other one, and the common coupling component and additives. On the other hand, some kinds of coupling components may be dispersed into separate layers, and in each layer are incorporated the same diazo compound and additives as in every other layer. In this case, individual color-producing units are constituted with a coupling component different from each other one, and the common diazo compound and additives. In any case, each color-producing unit is constituted with one or more kind of diazo compound, one or more kind of coupling component and other additives which are combined so as to produce a color of hue different from that obtained in every other color-producing unit.

The term "photo-decomposable diazo compounds" as used in the present invention refers mainly to aromatic diazo compounds, including aromatic diazonium salts, diazosulfonate compounds, diazoamino compounds and the like. The photo-decomposable diazo compounds are illustrated below, citing diazonium salts as typical examples.

In general, the wavelength at which diazonium salts undergo photolysis are said to be the wavelengths of their respective absorption maximum. In addition, the absorption maximum wavelength of a diazonium salt is known to vary between about 200 nm about 700nm according to its chemical structure(Takahiro Tsunoda & Tsugio Yamaoka, Nippon Shashin Gakkaishi, vol. 29(4), pp. 197-205 (1965), the title of which means "Photolysis of light-sensitive diazonium salts and chemical structures thereof", can be referred to). Namely, when diazonium salts are employed as a photo-decomposable compound, they decompose upon exposure to light of wavelengths specified depending on their respective chemical structures, and the hue of a dye to be produced by coupling reaction can be varied by using the diazonium salts of a modified chemical structure even when the same coupling component is used. Accordingly, diazonium salts can be used to advantage.

The diazonium salts are compounds represented by the general formula of ArN₂⁺ X⁻ (wherein Ar represents a substituted or unsubstituted aromatic moiety, N₂⁺ represents a diazonium group, and X⁻ represents an acid anion).

In a preferred embodiment of the present invention, two or more of diazonium compounds differing in photolysis wavelength are used.

Specific examples of diazonium compounds having their respective photolysis wavelengths in the vicinity of 400 nm include 4-diazo-1-dimethylaminobenzene, 4-diazo-1-diethylaminobenzene, 4-diazo-1-dipropylaminobenzene, 4-diazo-1-methylbenzylamino benzene, 4-diazo-1-dibenzylaminobenzene, 4-diazo-1-ethylhydroxyethylaminobenzene, 4-diazo-1-diethylamino-3-methoxybenzene, 4-diazo-1-dimethylamino-2-methylbenzene, 4-diazo-1-benzoylamino-2,5-diethoxybenzene, 4-diazo-1-morpholinobenzene, 4-diazo-1-morpholino-2, 5-diethoxybenzene, 4-diazo-1-morpholino-2,5-dibutoxybenzene, 4 diazo-1-anilinobenzene, 4-diazo-1-toluylmercapto-2,5-diethoxybenzene, 4-diazo- 1,4-methoxybenzoylamino-2,5-diethoxybenzene. Specific examples of compounds having their photolysis wavelengths in the range of 300 to 370 nm include 1-diazo-4(N,N-dioctylcarbamoyl)benzene, 1-diazo-2-octadecyloxybenzene, 1-diazo-4-(4-tert-octyl-phenoxy)benzene, 1-diazo-4-(2,4-di-tert-amylphenoxy)benzene,1-diazo-2-(4-tert-octylphenoxy)benzene, 1-diazo-5-chloro-2-(4-tert-octylphenoxy)benzene,1-diazo-2,5-bis-octadecyloxybenzene, 1-diazo-2,4-bis-octadecyloxybenzene, 1-diazo-4-(N-octylteuroylamino)benzene. Photolysis wavelengths of the aromatic diazonium compounds represented by the above-cited examples can be changed over a wide range by replacing their individual substitutent groups by other suitable groups.

Specific examples of acid anions include CₙF₂ₙ₊₁COO ⁻(n= an integer of 3 to 9),
CₘF₂ₘ₊₁SO₃⁻ (m= an integer of 2 to 8),
(CℓF_{2ℓ+1}SO₂)₂CH⁻(ℓ=an integer of 1 to 18),

Diazosulfonate compounds which can be used in the present invention are those represented by the following general formula: (wherein R₁ represents an alkali metal, or an ammonium compound; R₂, R₃, R₅ and R₆ each represents a hydrogen atom, a halogen atom, an alkyl group, or an alkoxyl group; and R₄ represents a hydrogen atom, a halogen atom, an alkyl group, an amino group, a benzoylamido group, a morpholino group, a trimercapto group or a pyrrolidino group).

Many compounds are known as such diazosulfonates, and can be obtained by treating the corresponding diazonium salts with a sulfite.

Preferred examples of diazosulfonate compounds include benzenediazosulfonates having such a substituent group as 2-methoxy, 2-phenoxy, 2-methoxy-4-phenoxy, 2,4-dimethoxy, 2-methyl-4-methoxy, 2,4-dimethyl, 2,4,6-trimethyl, 4-phenyl, 4-phenoxy, 4-acetoamide, or so on; and benzenediazosulfonates having such a substituent group as 4-(N-ethyl-N-benzylamino), 4-(N,N-dimethylamino), 4-(N,N-dimethylamino), 4-(N,N-diethylamino)-3-chloro, 4-pyrrolidino-3-chloro, 4-morpholino-2-methoxy, 4-(4ʹ-methoxybenzoylamino)-2,5-butoxy, 4-(4ʹ-trimercapto)-2,5-dimethoxy, or so on. When these diazosulfonoate compounds are used, it is desired that optical exposure should be carried out before printing for the purpose of activation of the diazosulfonates.

Other diazo compounds which can be used in the present invention are diazoamino compounds. Specific examples thereof include those obtained by coupling a diazo group with dicyandiamide, sarcosine, methyltaurin, N-ethylanthranicacid-5-sulfonic acid, monoethanolamine, diethanolamine or guanidine.

A developing agent to be combined with diazo compounds which can be used in the present invention is a coupling components which forms dyes by coupling with the diazo compounds (diazonium salts).

As examples of such a developing agent, mention may be made of not only 2-hydroxy-3-naphthoic acid anilide, but also those described in Japanese Patent Application (OPI) No. 144678/87 (=GB 8627461), including resorcin.

Also, image with arbitrary hue can be formed by the combined use of two kinds or more of these coupling components. As the coupling reaction of the diazo compounds with the coupling components is helped to take place in a basic atmosphere, a basic substance may be contained in a color-producing unit layer.

Suitable basic substances include those soluble slightly or insoluble in water, and substances capable of producing an alkali upon heating. As examples of such substances, mention may be made of inorganic and organic ammonium salts, organic amines, amides, urea and thiourea, derivatives of these ureas, thiazoles, pyrroles, pyrimidines, piperazines, guanidines, indoles, imidazoles, imidazolines, triazoles, morpholines, piperizines, amidines, formamidines, pyridines, and other nitrogencontaining compounds. Specific examples of the above compounds are described, e.g., in Japanese Patent Application(OPI) No. 291183/86.

Two or more basic substances may be used.

On the other hand, a basic dye precursor to be used in combination with a color developing agent in the color-producing unit of the present invention may be any compound provided that it can produce a color by donating an electron or accepting a proton of an acid or the like. In general, however, compounds of the kind which are nearly colorless, have a specified moiety, such as lactone, lactam, sultone, spiropyran, ester or amide and undergo the ring-opening or bond cleavage of the partial skeletons set forth above when brought into contact with a color developing agent are employed. Specific examples of such basic dye precursors include Crystal Violet lactone, benzoyl leuco Methylene Blue, Malachite Green lactone, Rhodamine B lactam, 1,3,3-trimethyl-6ʹ-ethyl-8ʹ-butoxyindolinobenzospiropyran, and so on.

As examples of a color developing agent to be used in combination with the foregoing basic dye precursors, mention may be made of phenol compounds, organic acids or metal salts thereof, oxybenzoates, and so on. A preferred melting point of a color developing agent ranges from 50°C to 250°C, particularly from 60°C to 200°C. In particular, phenols and organic acids which have a melting point ranging from 60°C to 200°C and are slightly soluble in water are favored over others.

Specific examples of these color developing agents are described, e.g., in Japanese Patent Application(OPI) No. 291183/86.

Materials which take part in the above-described color-producing reactions may be used in a form of a dispersion, or some of them may be used in a microencapsulated condition, if desired. From the standpoints of ensuring freshness keeping property through prevention of contact between a color-forming agent and a color-developing agent at ordinary temperatures (prevention of fog), and controlling the sensitivity concerning color production so that the color-producing reaction may take place by application of an intended quantity of thermal energy, it is of a great advantage to employ the microencapsulating technique described below.

Microcapsules preferably employed in the present invention have a microcapsule wall of such a property as to prevent the contact between substances present inside and outside the wall at ordinary temperatures through its insulation function, but to lower its permeability barrier to some of the substances only while it is heated to a temperature higher than a prescribed one. The microcapsule wall of this kind is disclosed in our previous applications, and a permeation starting temperature can be freely controlled by properly chosing a capsule wall material, a capsule core material, and additives. In this case, the permeation starting temperature corresponds to the glass transition point of the capsule wall (as described, e.g., in Japanese Patent Applications (OPI) Nos. 91438/86, 190886/84 and 242094/85.

For controlling the intrinsic glass transition point of a capsule wall, it is necessary to change the kind of a capsule wall-forming agent. Particulary preferred examples of capsules include a polyurea capsule, a polyurethane capsule, a polyurea-polyurethane mixture capsule, an urea-formaldehyde capsule, a capsule made of a mixture of polyurea and another synthetic resin, inside which some synthetic resin is contained as one of core materials, a capsule made of a mixture of polyurethane and another synthetic resin, a polyester capsule, a polyamide capsule, and the like. Microencapsulation methods and materials and compounds to be used therein are described in U.S. Patent 3,726,804 and 3,796,696.

A diazo compound, a coupling compound, and a basic substance may be incorporated into microcapsules as cited above, independently or as a combination of two or more thereof. The color-producing layer containing a combination of a diazo compound and a coupling compound as a color-producing unit can be formed using the thus microencapsulated compounds. Also, a basic dye precursor and a color developing agent may be incorporated into the above-described microcapsules, independently or in combination, and using the thus obtained microcapsules can be formed a color-producing layer containing a combination of a basic dye precursor and a color developing agent as a color-producing unit. These ingredients may be dissolved in an organic solvent or dispersed therein the form of fine particles prior to microencapsulation.

Microcapsules can be formed by the use of an emulsion containing an ingredient to be microencapsulated in a concentration of 0.2 wt % or more.

In forming a color-producing layer containing a combination of a diazo compound and a coupling component as a color-producing unit, it is desirable to use the coupling compound and a basic substance in amounts of 0.1 to 10 parts by weight and 0.1 to 20 parts by weight, respectively, per 1 part by weight of the diazo compound. On the other hand, in forming another color-producing layer containing a combination of a basic dye precursor and a color developing agent as a color-producing unit, the color developing agent is preferably used in an amount of 0.3 to 160 parts by weight, particularly 0.3 to 80 parts by weight, per 1 part by weight of the basic dye precursor.

In the present invention, a color-producing assistant can be used.

Color-producing assistants which can be used in the present invention are those which can increase a color density of the image printed by application of heat, or can contribute to a drop in the lowest possible temperature for color production. More specifically, they can lower the melting points of coupling compounds, alkalis, basic dye precursors, color developing agents, diazo compounds, etc., or the softening points of capsule walls, whereby such a condition as to facilitate the reaction among diazo, alkaline and coupling compounds, or the reaction between basic dye precursors and color developing agents, can be created.

Suitable color-producing assistants are phenol compounds, alcoholic compounds, amide compounds, sulfonamide compounds and so on. Specific examples of these compounds include p-tert-octylphenol, p-benzyloxyphenol, p-oxybenzoic acid phenyl ester, carbanilic acid benzyl ester, carbanilic acid phenetyl ester, hydroquinone dihidroxyethyl ether, xylylene diol, N-hydroxyethyl-methanesulfonic acid amide, N-phenyl-methanesulfonic acid amide. These compounds may be contained in the core substance of microcapsules, or be present outside the microcapsules.

In the heat sensitive material of the present invention, pigments, such as silica, barium sulfate, titanium oxide, aluminium hydroxide, zinc oxide or calcium carbonate, styrene beads, or fine powder of urea-melamine resin or the like can be used for the purpose of prevention of sticking to a thermal head, and improvement in writing facility.

Also, metallic soaps can be used for the prevention of sticking phenomenon. A coverage of such additives is appropriately 0.2 to 7 g/m².

In preparing the heat sensitive material of the present invention, a suitable binder can be used for coating.

Suitable examples of binders which can be used include polyvinyl alcohol, methyl cellulose, carboxymethyl cellulose, hydroxypropyl cellulose, gum arabic, gelatin, polyvinyl pyrrolidone, casein, styrene-butadiene latex, acrylonitrile-butadiene latex, and various kinds of emulsions of polyvinylacetate, polyacrylic acid esters and ethylene-vinylacetate copolymers. Such a binder is used at a coverage of 0.5 to 5 g/m² on a solids basis.

In addition to the above-described ingredients, an acid stabilizer, such as citric acid, tartaric acid, oxalic acid, boric acid, phosphoric acid, pyrophosphoric acid, etc., can be added to the heat sensitive material of the present invention.

In the case where the microencapsulation method is not employed, it is to be desired that diazo compounds, coupling compounds, basic dye precursors, color developing agents and so on should be used in the form of a solid dispersion prepared with a sand mill or the like. Herein, these ingredients are dispersed into separate solutions of water-soluble high polymers. As examples of water-soluble high polymers used preferably, mention may be made of those employed for the microencapsulation described above. A suitable concentration of such a water-soluble high polymer in each solution is 2 to 30 wt%, and each ingredient, such as a diazo compound, a coupling component, a basic substance, a basic dye precursor or a color developing agent, is added to the water-soluble high polymer solution so as to amount to 5 to 40 wt% therein.

A preferred size of particles dispersed is 10 microns or less.

An image recorded in the heat sensitive material of the present invention can be observed from one side as transmitted image or reflected image. In the latter case, the image is not clear since the back side is seen through the background area. Therefore, a white pigment may be added to a heat sensitive layer, or a layer containing a white pigment may be additionally provided. In both cases, it is effective to add a white pigment to the outermost layer located on the opposite side of the recorded-image observation. Suitable examples of white pigments include talc, calcium carbonate, calcium sulfate, magnesium carbonate, magnesium hydroxide, alumina, synthetic silica, titanium oxide, barium sulfate, kaolin, calcium silicate and urea resins.

A preferred coverage of a heat sensitive layer ranges from 3 to 20 g/m², particularly from 5 to 15 g/m². When the coverage is below 3 g/m² satisfactory sensitivity can not be obtained, whereas coverages beyond 20 g/m² can not contribute to improvement of image quality and become unfavorable in respect of production cost.

Now, a transparent support to be used in the present invention is illustrated below.

The term "transparent support" as used herein is intended to include films of polyesters such as polyethylene terephthalate, polybutylene terephthalate; cellulose derivative films like a cellulose triacetate film, polyolefin films such as a polystyrene film, a polypropylene film, a polyethylene film. These films may be used independently or in a laminated form.

A preferred thickness of such a transparent support is within the range of 20 to 200 microns, particularly 50 to 100 microns.

A subbing layer which can be employed in the present invention functions so as to heighten the adhesiveness between the transparent support and the heat sensitive layer. As a material for forming the subbing layer, mention may be made of gelatin, synthetic high polymer latexes and nitrocellulose. A preferred coverage of the subbing layer ranges from 0.1 to 2.0 g/m², particularly from 0.2 to 1.0 g/m². When the coverage is below 0.1 g/m², adhesion of the heat sensitive layer to the support is insufficient, whereas even when it is increased beyond 2.0 g/m², the adhesion power attains saturation to bring about only increase in cost.

It is to be desired that the subbing layer should be hardened with a hardener,because it sometimes swells in water contained in the heat sensitive layer coated thereon to cause deterioration of the image formed in the heat sensitive layer.

As examples of hardeners which can be used in the present invention, mention may be made of:
(1) active vinyl-containing compounds, such as divinylsulfone, N,Nʹ-ethylenebis(vinylsulfonylacetamide), 1,3-bis(vinylsulfonyl)-2-propanol, methylenebismaleimide, 5-acetyl-1,3-diacryloyl-hexahydro-s-triazine, 1,3,5-triacryloyl-hexahydro-s-triazine, 1,3,5-trivinylsulfonyl-hexahydro-s-triazine,
(2) active halogen-containing compounds, such as sodium salt of 2,4-dichloro-6-hydroxy-s-triazine, 2,4-dichloro-6-methoxy-s-triazine, sodium salt of 2,4-dichloro-6-(4-sulfoanilino)-s-triazine, 2,4-dichloro-6-(2-sulfoethylamino)-s-triazine, N,Nʹ-bis(2-chloroethylcarbamyl)piperazine,
(3) epoxy compounds, such as bis(2,3-epoxypropyl)methylpropylammonium-p-toluenesulfonate, 1,4-bis(2ʹ,3ʹ-epoxypropyloxy)-butane, 1,3,5-triglycidylisocyanurate, 1,3-diglycidyl-5-(α-acetoxy-β-oxypropyl)isocyanurate,
(4) ethyleneimino compounds, such as 2,4,6-triethylene-s-triazine, 1,6,-hexamethylene-N,Nʹ-bisethyleneurea, bis-β-ethyleneiminoethylthioether,
(5) methanesulfonate compounds, such as 1,2-di(methanesulfonoxy)ethane, 1,4-di(methanesulfonoxy)butane, 1,5-di(methanesulfonoxy)pentane,
(6) carbodiimide compounds, such as dicyclohexylcarbodimide, 1-cyclohexyl-3-(3-trimethylaminopropyl)carbodiimido-p-triethanesulfonate, 1-ethyl-3-(3-dimethylaminopropyl)carbodiimide hydrochloride,
(7) isooxazole compounds, such as 2,5-dimethylisooxazole perchlorate, 2-ethyl-5-phenylisooxazole-3-sulfonate, 5,5ʹ-(p-phenylene)bisisooxazole,
(8) inorganic compounds, such as chrome alum, boric acid, zirconium salt, chromium acetate,
(9) dehydrating condensation type peptide reagents such as N-carboethoxy-2-isopropoxy-1,2-dihydroquinoline, N-(1-morpholinocarboxy) 4-methylpyridinium chloride, and active ester compounds such as N,Nʹ-adipolyldioxydisuccinimide, N,Nʹ-terephthaloyl-dioxydisuccinimide, and
(10) isocyanates, such as toluene-2,4-diisocyanate, 1,6-hexamethylenediisocyanate.
(11) aldehydes such as glutaric aldehyde, glyoxal, dimethoxy urea, 2,3-dihydroxy-1,4-dioxane and the like.

Among these hardeners, especially aldehydes such as glutaric aldehyde, or 2,3-dihydroxy-1,4-dioxane, and boric acid are preferable.

Such a hardener is added in a proportion ranging from 0.20 to 3.0 wt% to the weight of the materials to constitute the subbing layer. A proper amount to be added can be selected depending on the coating method and the intended degree of hardening.

When the addition amount of a hardener is below 0.20 wt%, sufficient hardening can not be achieved however long the time elapsed is, and therefore the subbing layer swells upon coating of the heat sensitive layer, whereas when the hardener is added in a concentration higher than 3.0 wt% the hardening proceeds too fast, and therefore the adhesiveness between the subbing layer and the support is lowered to result in peeling of the subbing layer from the support in the form of a film.

According to the hardener used, the pH of a coating solution for the subbing layer can be rendered alkaline by the addition of sodium hydroxide or the like, or acidic by the addition of citric acid or the like, if needed.

Further, a defoaming agent can be added in order to eliminate foam generated upon coating, and a surface active agent can also be added in order to level the surface of the coating solution in a good condition so as to prevent coating streaks.

Furthermore, an antistatic agent can be added, if needed.

Before coating of the subbing layer, the surface of a support is preferably subjected to an activation processing according to known methods. As a method for the activation processing, mention may be made of an etching processing with an acid, a flame processing with a gas burner, a corona processing or glow discharge processing. From the viewpoint of cost or simplicity, corona discharge processing described in U.S.Patents 2,715,075 2,846,727, 3, 549,406 and 3,590,107, and so on are employed to the greatest advantage.

An overcoat layer can be provided on the heat sensitive layer of the present invention for a chief purpose of imparting water-resisting and scratch-resisting properties. As for the materials to constitute the over coat layer, polyvinyl alcohol, silicon-denatured polyvinyl alcohol, gelatin, a styrene-maleic anhydride copolymer or starch can be used as a binder, individually or as a mixture, and hardener similar to those usable in the foregoing subbing layer, or borax, boric acid, colloidal silica or the like is preferably employed.

Also, a white pigment, such as kaolin, calcium carbonate, titanium oxide, barium sulfate, zinc oxide, magnesium oxide, clay or the like, can be added to the overcoat layer for the purposes of increasing the whiteness of white areas of the recorded image and preventing the adhesion to a thermal head upon printing.

In addition, the whiteness of white areas of the recorded image can be further increased by adding a small amount of brightening agent or coloring dye to the overcoat layer. Moreover, the overcoat layer can be dyed uniformly with an appropriate dye so that the background may have a desired hue, other than white.

A preferred coverage of the overcoat layer ranges from 0.3 to 5 g/m², particularly from 0.5 to 4 g/m².

When the coverage is below 0.3 g/m², sufficient water resistance and scratch resistance cannot be impart to the heat sensitive material, whereas when it is increased beyond 4 g/m² excess energy is required for printing.

Coating compositions prepared in accordance with the present invention are coated using a dip coating process, an air knife coating process, a curtain coating process, a roller coating process, a doctor coating process, a wire bar coating process, a slide coating process, a gravure coating process or an extrusion coating process, using a hopper e.g. as described in U.S. Patent 2,681,294. Two or more of different coating compositions can be coated simultaneously, if desired, using methods described in U.S. Patents 2,761,791, 3,508,947, 2,941,898 and 3,526,528, Yuji Harasaki, Coating Kogaku (which means "Coating or Engineering"), p. 253, Asakura Shoten (1973). An appropriate method can be chosen from the above-cited ones depending on intended coverage, coating speed, and other factors.

The coating compositions thuse used may also include an appropriate pigment dispersing agent, a viscosity increasing agent, a fluidity modifying agent, a defoaming agent, a foam inhibitor, a mold lubricant or a coloring agent, as they have no adverse influences upon the characteristics of the material.

The heat sensitive material of the present invention can be employed as a sheet for high-speed recording in facsimiles and printers for electronic computers. In high-speed recording, differing from the recording with general type facsimiles and printers, it is desired that an apparatus equipped with a so-called double thermal head, which enables simultaneous heat recording on both sides, should be used. On the other hand, after recording on one side with a conventional single thermal head, recording may be carried out again on the other side of the sheet made to turn back facing its back side upward. In any case, as diazo compounds are used as color-forming component, additional incorporation of an exposure zone for the photolysis of the diazo compounds in a recording apparatus is advantageous from the standpoints of ensuring keeping quality of the produced image and increasing the numbers of producible hues.

Arrangements of printing heads and exposure zones are classified roughly into two types. In one type, after printing is carried out once, the recording sheet is subjected to optical exposure for photolysis; after this exposure, the recording sheet is turned back to the place where the printing was once carried out through a sending mechanism for the recording sheet in such a condition that the recording sheet waits for printing on the intended area thereof; and further such operations are repeated so that the printing and the optical exposure are carried out again, in this order, and then the recording sheet is turned back to the place for printing, this is a so-called one-head multi-scanning method. In the other type, a recording apparatus equipped with recording heads in the same numbers as those of colors to be recorded and exposure zones arranged between each adjacent recording heads is used; this is a multihead once-scanning method. Those two types may be used in combination, if needed. In addition, thermal energy to be supplied to a recording head may be changed, if needed. As for the light sources for photolyses, on the other hand, various kinds of light sources can be used, provided that they can be emit light of desired wavelengths. For instance, various kinds of fluorescent lamps, a xenon lamp, a xenon flash lamp, mercury lamps in which mercury vapor is enclosed at various pressures, a flash for photograph-taking or a strobe can be used.

In order to make the photofixation zone compact, a light source part and an exposure part may be set in separate positions, and these parts may be connected with optical fiber.

According to circumstances, a multicolor sample can be obtained in such a manner that a recording material on which printing was once done may be placed under sun light, a fluorescent lamp or the like, whereby achieving fixation by mainly utilizing light in the visible region, and then subjected to printing once more.

The present invention will now be illustrated in more detailed by reference to the following examples, wherein all parts are by weight unless otherwise indicated.

### Preparation of Diazo Capsule Solution (A):

The above-described ingredients were mixed, and added to an aqueous solution prepared by mixing 63 parts of a 8 wt% aqueous solution of polyvinyl alcohol and 100 parts of distilled water. The resulting mixture was converted to an emulsion having a mean particle size of 2 microns by a dispersion treatment at 20°C. The stirring of the emulsion was allowed to continue for 3 hours at 40°C.

Thereafter, the emulsion was cooled to 20°C and thereto was added 100 cc of an ion exchange resin (Amberlite IR-120B,registered trade mark, product of Rohm & Haas Co.). The mixture was stirred for one hour, and then passed through a filter to recover the resin and absorbed unencapsulated compounds. Thus, the capsule solution (A) was obtained.

### Preparation of Diazo Capsule Solution (B):

The above-described ingredients were mixed, and added to a mixture obtained by mixing 63 parts of a 8 wt% aqueous polyvinyl alcohol and 100 parts of distilled water. The resulting mixture was subjected to the same treatments as those for preparing the capsule solution (A) to result in formation of the capsule solution (B).

### Preparation of Coupler/Base Dispersion (A):

The above-described ingredients were mixed, and dispersed using a sand mill, Dyno Mill; trade name, product of Willy A Bachofen AG, Switzerland, and thereby was prepared a dispersion having a mean particle size of 3 microns.

### Preparation of Coupler/Base Dispersion (B):

The above-described ingredients were mixed, and subjected to the same treatments as those for preparing the coupler/base dispersion (A), and thereby was obtained the coupler/base dispersion (B).

### Preparation of Color-producing Assistance Dispersion:

28 parts of the color-producing assistant illustrated below: and 138 parts of a 4 wt% water solution of polyvinyl alcohol were mixed, and dispersed with a Dyno Mill (trade name, product of Willy A Bachofen AG) sand mill. Thus, a dispersion having a mean particle size of 3 microns was obtained.

### Preparation of Capsule Solution (C):

Basic Colorless Dye Precursor (Blue 200, produced by YAMADA KAGAKU K.K.) illustrated below:

The above-described ingredients were mixed, and added to a water solution prepared by mixing 100 parts of a 8 wt% water solution of polyvinyl alcohol and 40 parts of distilled water. The resulting mixture was converted to an emulsion having a mean particle size of 1 micron by a dispersion treatment at 20 C. The stirring of the emulsion was allowed to continue for 3 hours at 40 C to produce the capsule solution (C).

### Preparation of Capsule Solution (D):

The capsule solution (D) was prepared in the same manner as the capsule solution (C), except that the following compound (CIBA Pergascript Red I-6-B) was used as the basic colorless dye precursor:

### Preparation of Color Developing Agent Emulsified Dispersion:

The color developing agents (a), (b) and (c), illustrated below, were dissolved in amounts of 8 parts, 4 parts and 30 parts respectively, into a mixture of 8 parts of 1-phenyl-1-xylylethane and 30 parts of ethyl acetate. The resulting solution was admixed with a water solution consisting of 100 parts of a 8 wt% of water solution of polyvinyl alcohol, 150 parts of water and 0.5 part of sodium dodecylbenzenesulfonate to be converted to an emulsified dispersion having a mean particle size of 0.5 micron.

### Example 1

### Preparation of Recording Sheet A

With stirring were mixed 5.0 parts of the capsule solution (C), 10.0 parts of the emulsified dispersion of color developing agents, and 5.0 parts of distilled water. Thus, a coating composition A was prepared.

Separately, 4.9 parts of the capsule solution (A), 0.2 part of a 5 wt% water solution of hydroquinone, 3.7 parts of the coupler/base dispersion (B), and 7.4 parts of the color-producing assistant dispersion were mixed with stirring to prepare a coating composition B.

A 75µ-thick polyethylene terephthalate film which had received a biaxial streching treatment was used as a transparent support, and subjected to a double corona charging treatment. Thereafter, the coating composition A was coated on one side (side A) of the transparent support, and dried, while the coating composition B was coated on the other side (side B), and dried. The dry coverages were both 12 g/m². On each coated composition was provided a 2µ-thick protective layer having the following composition to obtained a recording sheet A.

### Composition of Protective Layer

Silica-denatured Polyvinyl Alcohol (PVA R2105), produced by KURARE K.K.) 1 part (on solids basis)
Colloidal Silica (Snowtex 30, produced by NISSAN KAGAKU K.K.) 1.5 parts (on solids basis)
Zinc Stearate (Hydolin Z-7, produced by CHUKYO YUSHI K.K.) 0.2 part (on solids basis)
Paraffin Wax (Hydolin P-7, produced by CHUKYO YUSHI K.K.) 0.02 part (on solids basis)

Heat was randomly applied for 1 second to several spots on each surface of the thus obtained recording sheet using a block heated to 100°C, then both sides of the recording sheet were exposed to light to carry out photofixation. The resultant sheet was observed from one side, and thereby underwent visual evaluation. The spots heated on the side A produced a clear cyan color, those on the side B a clear yellow color, and those on both sides a clear green color. The color separation among these colors was good. A Ricop of Super Dry Model 100 exposure machine of Ricoh Co., Ltd, was used for photofixation.

### EXAMPLE 2

### Preparation of Recording Sheet B

The coating compositions A and B were prepared in the same manners as those described in Example 1, respectively. In addition, the coating composition C was prepared by mixing with stirring, 4.9 parts of the capsule solution (B), 0.2 part of a 5 wt% water solution of hydroquinone, and 3.7 parts of the coupler/base dispersion (A).

The coating composition A was coated on one side (Side A) of the same transparent support as used for the recording sheet A, while on the other side (side CB) were coated the coating composition C, a composition for an interlayer, which was the same as the foregoing protective layer had, and the coating composition B, in this order. Dry coverages of the coating compositions A,B and C were all 12 g/m², and that of the interlayer was 2 g/m². Further, a protective layer having the same composition as in Example 1 was provided on each side to prepare the recording sheet B.

Heat was randomly applied for 1 second to several spots on each surface for this obtained recording sheet using a block heated to 100 C. The resultant sheet produced a cyan color on the side A, a yellow color on the side CB and a green color on both sides where the cyan coloring and the yellow coloring were overlapped.

After 10 seconds' exposure with a Ricopy Super Dry Model 100 exposure equipment at a wavelength of 400-430 nm, the recording sheet was heated for 1 second with a block heated to 120°C to result in magenta coloration on the heated spots.

In analogy with Example 1, the recording sheet produced yellow color and cyan color on both sides, respectively, by printing at a low temperature prior to optical exposure. After photolysis of the remaining long wavelength light absorbing diazo compounds by optical exposure, the resultant recording sheet was subjected to printing at a somewhat higher temperature than before to result in magenta coloration. Thus, when the recording sheet was observed from one side, cyan, magenta, yellow, blue (cyan+magenta), green (cyan+yellow), red (yellow+magenta) and black (cyan+magenta+yellow) color images were found therein. These images were all clear, free from unwanted color stain and blur.

### EXAMPLE 3

### Preparation of Recording Sheet C

The coating composition B and C were prepared in the same manners as those described in Example 2, respectively. In addition, the coating composition D was prepared by mixing, with stirring, 5.0 parts of the capsule solution (D), 10.0 parts of the emulsified dispersion of the color developing agents, and 5.0 parts of water.

On one side (Side AB ) of the same transparent support as used for the recording sheet A were coated the coating composition A, a composition for an interlayer, which was the same as the foregoing protective layer had, and the coating composition B, in this order, while the coating composition D was coated on the other side (Side D). Dry coverages of the coating compositions A, B and D were all 12 g/m², and that of the interlayer was 2 g/m².

Further, a protective layer having the same composition as in Example 1 was provided on each side to prepare the recording sheet C.

The recording sheet C was made to produce colors using the same process as in Example 2 to provide the same color images as the recording sheet B. That is, when the sheet was observed from one side, images of cyan, magenta, yellow, blue(cyan+magenta), green(cyan+yellow), red(yellow+magenta) and black(cyan+magenta+yellow) colors were found therein. These images were all clear, free from undesirable stain and blur.

## Claims

1. A multicolor heat-sensitive recording material which comprises a transparent support(s) having two or more color-producing unit layers differing in hue of the produced color, characterised in that said layers are arranged so that at least one unit layer (C, M and Y) is provided on each side of the support, said unit layers being each constituted by one or more color-producing unit layer containing a combination of (a) precursor of a basic dye with (b) a color-developing agent as a color-producing unit, and one or more color-producing unit layer containing a combination of a (c) diazo compound with (d) a coupling component for the diazo compound as a color-producing unit.

2. A multicolor heat-sensitive recording material as claimed in Claim 1, wherein the color-producing unit layers are comprised of three layers (C, M and Y) producing cyan coloring, magenta coloring and yellow coloring respectively.

3. A multicolor heat-sensitive recording material as claimed in Claim 2, wherein the magenta color-producing unit layer (M) and/or yellow color-producing layer (Y) contains a combination of diazo compound with a coupler as a color-producing unit.

4. A multicolor heat-sensitive recording material as claimed in Claim 1, 2 or 3, wherein at least one component of the basic dye precursor and the color-developing agent, and at least one component of the diazo component and the coupler are microencapsulated.

5. A multicolor heat-sensitive recording material as claimed in Claim 4, wherein at least both the basic dye precursor and diazo compound are microencapsulated.

6. A multicolor heat-sensitive recording material as claimed in any preceding claim, wherein the color-developing agent (b) melts at a temperature of 50 to 250°C.

7. A method of forming a multicolor image, which comprises imagewise heating a material as claimed in any preceding claim from one or both side of the support.

8. A method as claimed in Claim 7, wherein the image produced is fixed by overall exposure to light.

9. A method as claimed in Claim 8, wherein the sheet is then subjected to imagewise heating at a higher temperature than the first heating, to produce a different hue image.
